

# UNITED STATES PATENT OFFICE.

CHRISTOPHER F. WHITNEY, OF NEWTON, MASSACHUSETTS.

## ALUMINIUM ALLOY.

SPECIFICATION forming part of Letters Patent No. 501,553, dated July 18, 1893.

Application filed November 28, 1892. Serial No. 453,404. (No specimens.)

*To all whom it may concern:*

Be it known that I, CHRISTOPHER F. WHITNEY, of Newton, in the county of Middlesex and Commonwealth of Massachusetts, have

5 invented certain Improvements in Aluminium Alloys, of which the following description is a specification.

My invention consists in alloying aluminium with manganese and tungsten, in proportions of twelve per cent., or less, of each, to seventy-six per cent., or more of aluminium. This alloy is especially well adapted for use in making culinary vessels. I prefer to use no greater amount than twelve per cent., of

manganese and tungsten, but as small a quantity as one half of one per centum of each of those metals is of perceptible benefit in making an aluminium alloy.

What I claim is—

A metal alloy consisting of aluminium in 20 proportions of seventy-six per cent. or more and of manganese and tungsten in proportions of twelve per cent. or less of each.

CHRISTOPHER F. WHITNEY.

Witnesses:

A. J. BURROWS,  
T. J. CUNNINGHAM.